

No. 660,221.

Patented Oct. 23, 1900.

J. A. POTTER.

MANUFACTURE OF ORDNANCE AND PROJECTILES.

(Application filed Apr. 15, 1898.)

(No Model.)

2 Sheets—Sheet 1

Fig. 1.



Fig. 2.



Fig. 3.



*J. A. Potter*  
*J. B. Lemming*

John A. Potter  
by *Barrett* *Barrett*  
his atty.

No. 660,221.

Patented Oct. 23, 1900.

J. A. POTTER.

MANUFACTURE OF ORDNANCE AND PROJECTILES.

(Application filed Apr. 15, 1898.)

(No Model.)

2 Sheets—Sheet 2.

Fig. 4.



Fig. 5

Fig. 6.



WITNESSES

J. A. Potter  
G. B. Lemming

INVENTOR

J. A. Potter  
by Baker & Baker  
his atty

# UNITED STATES PATENT OFFICE.

JOHN A. POTTER, OF CLEVELAND, OHIO.

## MANUFACTURE OF ORDNANCE AND PROJECTILES.

SPECIFICATION forming part of Letters Patent No. 660,221, dated October 23, 1900.

Application filed April 15, 1898. Serial No. 677,660. (No model.)

*To all whom it may concern:*

Be it known that I, JOHN A. POTTER, of Cleveland, in the county of Cuyahoga and State of Ohio, have invented a new and useful Improvement in the Manufacture of Ordnance and Projectiles, of which the following is a full, clear, and exact description, reference being had to the accompanying drawings, forming part of this specification, in 10 which—

Figure 1 is a sectional elevation of one form of press constructed in accordance with my invention. Fig. 2 is an enlarged partial section of another form, showing the plungers in 15 depressed position. Fig. 3 is a horizontal section on the line III III of Fig. 2; and Figs. 4, 5, and 6 are partial sectional elevations showing other forms of the press.

My invention relates to the manufacture of 20 ordnance and projectiles, and is designed to provide an improved method therefor, whereby such articles may be cast without substantial piping or segregation in the interior of the casting.

25 To that end it consists in subjecting the molten metal to an end pressure until the outer shell is solidified, keeping the end portion hot and then subjecting the central end portion to a further pressure, thus preventing the fluid interior portion from piping and 30 from internal strains and segregation.

In the drawings, referring to the form of Figs. 1, 2, and 3, 2 represents a mold which is built up of interfitting steel plates, which 35 are preferably water-cooled by pipes or channels 3 and which are bolted together by pins or bolts 4, extending through slots cut in the edges of the sections. These slots are so arranged that they register in alternate plates, 40 the arrangement of the pins or bolts being clearly shown in Figs. 2 and 3. I show the mold as resting upon a base 5, carried upon the plunger of a hydraulic ram 6, carried centrally in the foundation of the machine and 45 arranged to lift the base-plate from the rollers 7, upon which the plate and mold are carried into position in the press. 8 are the side standards of the press, which form guides for a vertically-reciprocating cross-head 9, 50 secured to the plunger 10 of a hydraulic cylinder 11. This plunger 10 is hollow and

forms the cylinder for an inner ram or plunger 12, the reduced portion 13 of which extends through the cross-head and through a block 14, centrally secured to the cross-head, 55 which block fits neatly within the open upper end of the mold. The ram 13 extends through a cavity 15 in this block, to which powdered or granular material—such as sand, small shot, or similar material—may be fed through 60 openings 16. Below this cavity the block is cut out in its lower portion, so as to receive a steel ring 17, adapted to contain a plug 18 of refractory material, this plug being of about the same diameter as the ram or rod 13. I 65 provide at the sides of the cylinder 11 small lifting-cylinders 19, the rods of whose pistons are connected to the cross-head 9 and serve to lift the same after the operation is completed. Fluid-pressure is admitted to the interior of the hollow ram 10 through a tubular extension 20, extending through the top of its cylinder and secured to the ram, the fluid passing through a jointed pipe 21. The smaller ram 12 is lifted by a rod 22, extending 70 upwardly through the tubular extension to a piston 23 in an upper lifting-cylinder 24.

The operation is as follows: The mold, which has been suitably lined with a refractory material, as shown, being filled with molten steel 80 fluid pressure is admitted to the larger cylinder 11, thus forcing down the cross-head and pressure-block and subjecting the molten steel to a heavy hydraulic pressure. The inner ram 12 moves down with the plunger 10, 85 remaining at the same point in the outer plunger during this operation. As soon as the outer shell of metal next to the mold has chilled so that the metal cannot be further compressed in its outer portions fluid-pressure is admitted within the hollow plunger 10, thus forcing down the inner ram 13. This ram acting upon the refractory plug 18 forces this plug through the ring 17 into the central portion of the still liquid metal and subjects 90 the same to a heavy pressure. In order to prevent the plunger from entering and becoming embedded in the solidifying steel after it has forced down the refractory plug, it is lifted sufficiently to allow the granular material in the cavity of the pressure-block to feed down into the opening through the bot- 95 100

tom of the block, and the ram 13 then being forced down again acts through this intermediate material upon the interior partially-cooled body of the metal. This operation is 5 repeated as often as desirable. The ring 17 reduces the area upon which the smaller ram operates, and as the top of the ingot chills the ring becomes secured in place and fastened in and sustained by the castings and 10 sustains the intensified pressure upon the small ram and concentrates its power at the desired point. The gases will pass up into the cavity of the pressure-block and thence out through the filling-openings. The refractory plug being of non-conducting material tends to keep the central portion of the metal hot, and thus allows the compressive action of the inner plunger to be exerted thereon. The central piping and segregation of the 15 casting is thus prevented and an exceedingly strong homogeneous metal is obtained throughout it. I may obtain this successive pressure first upon the entire body of the metal and then upon its inner hotter portion 20 in many other ways. Thus in Fig. 4 I show a single ram 25, having secured to its lower end a pressure-block 26, the lower part of which is reduced in diameter and is surrounded by a series of rings or collars. The 25 lowermost ring 27 is provided with a central curved block 28, of refractory material, against the central part of which the end of the pressure-block abuts. Above this ring is an inner collar 29, surrounding the reduced portion of the block, and surrounding 30 this collar are two rings 30, the lower of which is composed of steel, while the upper is composed of zinc or some easily-fusible metal. The upper face of the zinc ring is in the same 35 plane as the top of the collar, and covering them both is an annular plate 31 of steel, above which is an inner zinc ring 32 and outer zinc ring 33, the ring 33 being of less thickness than the ring 32. When the ram is forced 40 down to bring the pressure upon the molten steel in the mold in this form, the block of refractory material will keep the central part of the steel hot, and the heat being conducted from the metal upwardly through the rings 45 and collars will gradually soften and melt the zinc ring 30. The outer shell of the casting having cooled during the softening of this ring the whole pressure of the ram is brought upon the block and its collar 29, which bearing 50 upon the refractory block will drive it down into the hotter metal and compress it. As the portions next to the outer shell congeal, thus preventing further downward movement of the collar, the heat will be conducted to the zinc rings 32 33, and these rings 55 will soften and melt, allowing the reduced part of the block to move down within the collar 29 and act upon the central portion of the molten metal. I am thus enabled to automatically concentrate the pressure which 60 is first brought upon the entire body of molten 65

metal upon its intermediate and central portions successively during the congealing of the casting, thus obtaining a solid compact metal.

In the form of Fig. 5 the rings 34 and 35, surrounding the reduced portion of the pressure-block above the collars 36 and 37, are of steel and are made in two or more parts, so that after the ram is depressed to bring the 70 pressure upon the molten metal the plunger may be lifted and a portion of these rings removed, so as to allow the block and intermediate collar to press upon the inner hotter portion of the metal, and when these are cooled 75 it may be again raised and the inner rings removed, after which the plunger is again depressed, and the block sliding down within the collars acts upon the central part only of the cooling metal.

In the form of Fig. 6 I employ in place of the steel pressure-block a block 38 of wood, such a lignum-vitæ, which may be provided in its lower face with a block of refractory material and may be provided with encircling 80 bands or hoops sunk in annular recesses to prevent crushing of the block. When this block is forced down into the steel, its portions around the refractory material will char and gradually burn away, so that the pressure will be applied to the central part of the molten metal, thus concentrating the pressure upon the hotter parts of the metal, as in the 85 previous forms.

I may carry out my process with a plain 90 solid steel block of shape shown in Fig. 6, this block being secured to the lower end of the plunger and fitting into the upper end of the mold-cavity by feeding in granular material, such as hot sand, and forcing this material down upon the cooling metal. As the outer shell cools more material is fed in and 95 will be forced down in the central hotter portions, so as to concentrate the pressure thereon, as before.

The advantages of my invention will be apparent to those skilled in the art. The compressive force is exerted throughout the entire cooling and solidifying of the steel, thus obviating the piping and internal strains 100 heretofore caused by the contraction of the interior fluid metal after the outer shell has solidified. The rapid cooling of the article is hastened by the great pressure and consequent close contact of the metal with the 105 mold, and a greater pressure may be exerted upon the interior of the article than could be carried by the mold were it not for the solidified shell surrounding the interior hot metal. The inner part of the article is kept hot by 110 the refractory plug or material, and the compressive action may thus be prolonged upon this part. The gases expelled from the steel by the great pressure brought thereon will 115 pass into the refractory lining and thence through the joints between the mold-sections.

The invention is applicable also to the mak-

ing of ingots, shafts, and other castings, and I intend to cover the same when used upon any casting apparatus.

Many changes may be made in the form and arrangement of the press and in the means for applying pressure to the inner hotter portion of the metal as the outer parts chill and harden without departing from my invention, since

10 What I claim is—

1. The method of making castings, consisting in subjecting molten metal in the mold to endwise pressure over a major portion of its area, keeping the central end portion hot, and 15 then compressing this central portion alone by further localized pressure after the har-

dening of the outer shell; substantially as described.

2. The method of making castings, consisting in subjecting molten metal in the mold to 20 endwise pressure over substantially the entire end portion; keeping the central end portion hot, and then compressing this central portion alone after the compression of the entire end portion; substantially as described. 25

In testimony whereof I have hereunto set my hand.

JOHN A. POTTER.

Witnesses:

J. C. JONES, Jr.,  
F. H. HART.